# EUROPEAN PATENT SPECIFICATION

(11) **EP 1 651 402 B1**
(45) Date of publication and mention of the grant of the patent: **26.01.2011**
(21) Application number: 04742205.0
(22) Date of filing: 23.07.2004
(51) Int. Cl.: B27K 3/36, B27K 5/00

(54) **TREATMENT OF THERMALLY MODIFIED WOOD**
BEHANDLUNG VON THERMISCH MODIFIZIERTEM HOLZ
TRAITEMENT DE BOIS THERMO-MODIFIE

(30) Priority: 25.07.2003 FI 20031103
(43) Date of publication of application: 03.05.2006
(73) Proprietor: Stora Enso Oyj, 00160 Helsinki (FI)
(72) Inventor: LAITINEN, Risto, FI-55420 Imatra (FI); KANKKUNEN, Mika, FI-55510 IMATRA (FI); LINDELL, Henry, FI-55800 Imatra (FI); LEHTOVUORI, Jukka, FI-44100 Äänekoski (FI); SILEN, Jouko, FI-11120 Riihimäki (FI); PÄNKÄLÄINEN, Saku, FI-48310 Kotka (FI)
(74) Representative: Svensson, Johan Henrik
(86) International application number: PCT/FI2004/000462
(87) International publication number: WO 2005/009700

(56) References cited:
- EP-A1- 0 327 215
- WO-A2-02/081159
- CALLUM A.S. ET AL.: 'The chemical modification of scots pine with succinic anhydrode or octenyl succinic anhydride' HOLZFORSCHUNG vol. 52, 1998, pages 427 - 433, XP002996213

## Description

The invention relates to a method for treating thermally modified wood, the product obtained with the method and the use of processing agents in conjunction with the method.

Thermal modification of wood means controlled thermal treatment of timber at a temperature above 100 °C so that the treatment improves the dimensional stability of the wood and reduces its equilibrium moisture content and moisture life. Other beneficial effects of thermal modification comprise increased decay resistance and reduced pitch secretion. On the other hand, thermal modification results in darkened wood and impaired bending and splitting resistance. Owing to its properties, thermally modified wood is applicable especially to constructions and furniture exposed to contact with outdoor air.

Thermal wood modifying techniques have been described in WO 95/31680, which focuses on control of the temperature difference between the outer surface and the interior of the wood during the temperature increase so as to prevent cracks in the wood. In this reference, the temperature difference is in the range 10-30 °C and this range is maintained roughly constant during heating. According to this reference, a corresponding controlled temperature difference in the range 10-30 °C between the wood interior and its outer surface can also be maintained during cooling of the wood, during which, unlike the heating process, the higher temperature prevails within the wood.

WO 94/27102 discloses an improved method for producing thermally modified wood, in which the wood treatment temperature is above 150 °C, the treatment being performed with the aid of steam. A weight loss of at least 3% of the wood occurs in the course of the treatment.

WO 01/53812 further describes a procedure for recognizing the thermal modification in wood by measuring the number of free radicals in the wood and by comparing this number with that of free radicals in corresponding untreated wood. The reference sets forth as a criterion for thermal modification that the number of free radicals in the wood should be at least 1.5-fold, preferably at least double compared to untreated wood.

WO 02/081159 discloses the use of various substances for protecting wood. EP 0 327215 discloses the use of certain ketene dimers for sizing unbleached fibers or undigested wood chips for use in building products. Callum A.S. et al.: 'The chemical modification of Scots Pine with succinic anhydrode or octenyl succinic anhydride' Holzforschung vol. 52, 1998, pages 427-433 discusses the use of octenyl succinic anhydride in the treatment of wood.

In the following, thermal wood modification or thermally modified wood implies that the wood meets the criteria of thermal wood modification or of thermally modified wood defined in respect of WO 01/53812 as cited above.

Despite the reduced equilibrium moisture content of thermally modified wood in moist outdoor air, it has now been found that such wood, when brought into direct contact with water or moist soil, absorbs water in abundance. Although thermal modification as such enhances the decay resistance of wood, especially long-term waterlogging still has a detrimental effect on the resistance of the wood. In addition, soaked wood material gets a markedly increased weight.

The object of the present invention is thus to provide a solution in order to prevent waterlogging of thermally modified wood. The invention is defined in the attached claims. The method of the invention comprises water-repellency treatment of thermally modified wood by means of a hydrophobic sizing agent reactive to cellulose. The treatment is preferably performed with a solution containing the hydrophobic sizing agent, followed by solvent evaporation by means of drying.

In accordance with the invention, it has been found that a size dissolved in a suittable organic solvent is readily absorbed into thermally modified wood, and this is due to the same fact as is waterlogging of wood, i.e. increased porosity of the wood structure. The preliminary tests conducted in accordance with the invention achieved a contact angle above 90 °, even above 100 °, between the surface of the treated wood and a water droplet deposited onto this, such an angle being an indication of high water repellence.

The entire wood material can be impregnated with the solution containing the sizing agent in order to achieve a constant size concentration. Optionally, the wood can be surface-treated by painting or by immerging it rapidly into an immersion basin, the surfaces of the piece of wood being treated throughout, while the size penetrates into the surface layers alone.

Sizing agents suitable for increasing the hydrophobicity of wood in accordance with the invention include sizing agents reactive with cellulose, the sizing being performed in the neutral or alkaline pH range. Such sizing agents comprise alkyl ketene dimers (AKD) and alkenyl succinic acid anhydrides (ASA) known in paper and board sizing, among other applications. The paper and board industry uses these sizes in the form of water emulsions, whereas they are most expedient in impregnating thermally modified wood of the invention when dissolved into an organic solvent, such as acetone. In terms of absorbability, the size solution is preferably diluted, with the size concentration in the solution being e.g. 0.01-5% by weight, preferably 0.05-0.2% by weight. However, the invention also allows for the use of a 100% AKD, ASA or similar size as such without any solvent, in the form of a concentrated solution, dispersion or emulsion, the medium of the dispersion or emulsion of the invention being e.g. water, and the proportion of sizing agent equalling the size concentrations in the solution mentioned above. AKD and ASA can further be jointly used when intermixed.

The used in the invention alkyl ketene dimers (AKD) sizes comprise a straight C₁₆-C₂₂ alkyl chain. AKD size preparations are available both in a solid and a liquid form.

ASA sizes used in the invention comprise a C₁₆-C₂₂ alkenyl chain.

In prior art, the article of C.A.S. Hill and S. Mallon in the Journal of Wood Chemistry and Technology, 18 (3), pages 299-311 (1998) explain chemical wood modification, in which one of the chemicals was 2-octene-1-yl succinic acid anhydride, which pertains to the ASA sizes, dissolved in pyridine. However, this was not a case of thermally modified wood, nor did it aim at increased hydrophobicity of the wood, but instead at increased dimensional stability and resistance of the wood and at an increased number of reactive functional groups in the wood by chemical means. The technique described in the article is thus associated with thermal wood modification rather than with wood hydrophobisation.

After the sizing and the evaporation of the solvent or emulsion or dispersion medium of the invention, the wood can be further processed by heating, e.g. by exposing it to a temperature in the range 100 - 140 °C for 15-60 minutes. The required heating depends on the sizing agent selected; preliminary tests indicate that such after-heating is almost insignificant in AKD sizing, whereas it improves the hydrophobicity obtained with ASA crucially.

The thermally modified wood of the invention treated as above is characterised in having been impregnated with a hydrophobic sizing agent reactive with cellulose, which makes the wood more water-repellent. The size has impregnated at least the surface layers of the piece of wood, so that the surfaces of the piece are protected by the size on all sides. The size may be evenly distributed throughout the wood, with the size concentration in the treated wood being approximately constant.

The invention further comprises the use of a hydrophobic size, such as AKD or ASA, in water-repellency treatment of thermally modified wood.

The invention is illuminated below by means of the following embodiment examples.

### Example 1

AKD size containing a C₁₆/C₁₈ alkyl chain was dissolved in acetone to a solubility of 0.1% by weight and thermal wood marketed under the name Thermowood was thoroughly impregnated with this solution. The wood was dried by evaporating the acetone solvent and the dried AKD treated wood was heated to 130 °C over periods of 15, 30 and 60 min., respectively. The water repellence of the wood was tested by a drop test, in which the contact angle formed by the water droplet placed on the wood and the wood itself was measured after contact periods of 1, 5 and 10 s., respectively. The bar chart in enclosed figure 1 shows the results of five samples, a reference sample (ref.), i.e. thermal wood not treated with AKD, AKD treated thermal wood, which had been dried but not subjected to a heating process, and AKD treated thermal wood, which had been dried and then heated to 130 °C over periods of 15, 30 or 60 minutes. The results show the hydrophilicity of wood not treated with AKD, appearing as a low contact angle, which further decreases rapidly as the contact is prolonged. Thermal wood treated with AKD yielded contact angles of approx. 90-100° , which indicated that the surface was water repellent and devoid of a tendency of water absorption into the wood. It also indicates that a heating treatment following the AKD sizing has only a marginal bearing on the hydrophobicity of the wood and that heating of excessive duration may have a negative impact.

### Example 2

The tests of example 1 were reproduced with the use of ASA containing a C₁₈-C₂₂-alkenyl chain in lieu of AKD. Using a process solution containing 0.1% of ASA dissolved in acetone, the contact angles of a water droplet were determined on dried and impregnated thermal wood as such or after heating treatments of 15, 30 or 60 minutes at 130 °C, at the end of contact periods of 1, 5 and 10 s. As in example 1, the reference (ref.) comprised a commercial unsized thermal wood as such. The results appear in the bar chart of figure 2 in the drawing. It appears that ASA sizing alone, without heating, does not achieve any marked improvement in the hydrophobicity of thermal wood, whereas excellent hydrophobicity appearing as an approx. 100° contact angle is achieved when ASA sized and dried thermal wood is additionally subjected to a short heating process.

## Claims

1. A method for treating thermally modified wood having the number of free radicals turned to at least 1.5-fold by the modification as compared to corresponding untreated wood, **characterised in that** a piece of the thermally modified wood is made water repellent by impregnating it with a hydrophobic sizing agent, which is reactive with cellulose, the sizing agent being an alkyl ketene dimer (AKD) with a straight C₁₆-C₂₂ alkyl chain and/or an alkenyl succinic acid anhydride (ASA) with a C₁₆-C₂₂ alkenyl chain, and at least when the sizing agent is ASA the treated wood is dried and then heated to a temperature of 100-140 °C for 15-60 minutes.

2. A method as defined in claim 1, **characterised in that** the wood is made water repellent by treating it with a solution or a dispersion containing a hydrophobic sizing agent and by removing the solvent or dispersion medium by means of drying.

3. A method as defined in claim 2, **characterised in that** the surfaces of a piece of wood are treated throughout with a solution or dispersion containing a sizing agent.

4. A method as defined in any of claims 2-3, **characterised in that** the sizing agent has been dissolved in an organic solvent, such as acetone.

5. A method as defined in any of claims 2-4, **characterised in that** the content of sizing agent in the process solution or dispersion is 0.01 - 5% by weight, preferably 0.05 - 0.2% by weight.

6. A piece of thermally modified wood obtainable by a method according to any of the preceding claims, **characterised in that** the wood has been impregnated with a hydrophobic sizing agent, which is reactive with cellulose and by means of which the wood has been made water repellent, said sizing agent being an alkyl ketene dimer (AKD) with a C₁₆-C₂₂ alkyl chain and/or an alkenyl succinic acid anhydride (ASA) with a C₁₆-C₂₂ alkenyl chain.

7. A piece of thermally modified wood as defined in claim 6, **characterised in that** the wood has been impregnated with the sizing agent to evenly distribute sizing agent throughout the wood.

8. Use of a hydrophobic size reactive with cellulose in the treatment of a piece of thermally modified wood having a number of free radicals turned to at least 1.5-fold by the modification as compared to corresponding untreated wood, the wood being impregnated with the size to make it water repellent, said size being an alkyl ketene dimer (AKD) with a straight C₁₆-C₂₂ alkyl chain and/or an alkenyl succinic acid anhydride (ASA) with a C₁₆-C₂₂ alkenyl chain, and at least when the sizing agent is ASA the treated wood is dried and then heated to a temperature of 100-140 °C for 15-60 minutes.

## Patentansprüche

1. Verfahren zum Behandeln von thermisch modifiziertem Holz, wobei die Anzahl von freien Radikalen durch die Modifikation auf wenigstens das 1,5-Fache erhöht ist im Vergleich zu entsprechendem unbehandelten Holz, **dadurch gekennzeichnet, dass** ein Stück des thermisch modifizierten Holzes wasserabweisend gemacht wird durch Imprägnieren des Holzes mit einem hydrophoben Leimungsmittel, welches mit Zellulose reaktionsfähig ist, wobei das Leimungsmittel ein Alkylketendimer (AKD) mit einer geraden C₁₆-C₂₂ Alkylkette und/oder einem Alkenylbernsteinsäureanhydrid (ASA) mit einer C₁₆-C₂₂ Alkenylkette ist, und wobei zumindest, wenn das Leimungsmittel ASA ist, das behandelte Holz getrocknet wird und dann für 15 bis 60 Minuten auf eine Temperatur von 100 bis 140 °C erhitzt wird.

2. Verfahren nach Anspruch 1, **dadurch gekennzeichnet, dass** das Holz wasserabweisend gemacht wird, indem es mit einer Lösung oder einer Dispersion behandelt wird, welche ein hydrophobes Leimungsmittel enthält, und in dem das Lösungs- oder Dispersionsmedium durch Trocknen entfernt wird.

3. Verfahren nach Anspruch 2, **dadurch gekennzeichnet, dass** die Oberflächen eines Holzstückes durchweg mit einer Lösung oder Dispersion behandelt werden, welche ein Leimungsmittel enthält.

4. Verfahren nach einem der Ansprüche 2 bis 3, **dadurch gekennzeichnet, dass** das Leimungsmittel in einem organischen Lösungsmittel, wie z.B. Azeton, gelöst worden ist.

5. Verfahren nach einem der Ansprüche 2 bis 4, **dadurch gekennzeichnet, dass** der Gehalt des Leimungsmittels in der Prozesslösung oder -dispersion 0,01 bis 5 Gewichtsprozent, vorzugsweise 0,05 bis 0,2 Gewichtsprozent, beträgt.

6. Thermisch behandeltes Holzstück, welches durch ein Verfahren nach einem der vorhergehenden Ansprüche erhältlich ist, **dadurch gekennzeichnet, dass** das Holz mit einem hydrophoben Leimungsmittel imprägniert worden ist, welches mit Zellulose reaktionsfähig ist, und mittels dem das Holz wasserabweisend gemacht worden ist, wobei das Leimungsmittel ein Alkylketendimer (AKD) mit einer C₁₆-C₂₂ Alkylkette und/oder einem Alkenylbernsteinsäureanhydrid (ASA) mit einer C₁₆-C₂₂ Alkenylkette ist.

7. Thermisch behandeltes Holzstück nach Anspruch 6, **dadurch gekennzeichnet, dass** das Holz mit dem Leimungsmittel imprägniert worden ist, um das Leimungsmittel gleichmäßig über das Holz zu verteilen.

8. Verwendung eines hydrophoben Leims, der mit Zellulose reaktionsfähig ist, in der Behandlung eines Stücks thermisch modifizierten Holzes, bei dem eine Anzahl von freien Radikalen durch die Modifikation auf wenigstens das 1,5-Fache erhöht ist im Vergleich zu entsprechendem unbehandelten Holz, wobei das Holz mit dem Leim imprägniert wird, um es wasserabweisend zu machen, wobei der Leim ein Alkylketendimer (AKD) mit einer geraden C₁₆-C₂₂ Alkylkette und/oder einem Alkenylbernsteinsäureanhydrid (ASA) mit einer C₁₆-C₂₂ Alkenylkette ist, und wobei zumindest, wenn das Leimungsmittel ASA ist, das behandelte Holz getrocknet wird und dann für 15 bis 60 Minuten auf eine Temperatur von 100 bis 140 °C erhitzt wird.

## Revendications

1. Procédé destiné à traiter du bois thermiquement modifié ayant le nombre de radicaux libres augmenté d'au moins 1,5 fois par la modification par rapport à un bois non traité correspondant, **caractérisé en ce qu'**un morceau du bois thermiquement modifié est rendu hydrofuge en étant imprégné d'un agent de collage hydrophobe, qui est réactif avec la cellulose, l'agent de collage étant un dimère d'alkyl cétène (AKD) ayant une chaîne alkyle en C₁₆-C₂₂ droite et/ou un anhydride d'acide alcényle succinique (ASA) ayant une chaîne alcényle en C₁₆-C₂₂, et au moins lorsque l'agent de collage est l'ASA, le bois traité est séché et ensuite chauffé à une température de 100 à 140°C pendant 15 à 60 minutes.

2. Procédé selon la revendication 1, **caractérisé en ce que** le bois est rendu hydrofuge en étant traité avec une solution ou une dispersion contenant un agent de collage hydrophobe et en retirant le milieu solvant ou de dispersion par séchage.

3. Procédé selon la revendication 2, **caractérisé en ce que** les surfaces d'un morceau de bois sont entièrement traitées avec une solution ou une dispersion contenant un agent de collage.

4. Procédé selon l'une quelconque des revendications 2 à 3, **caractérisé en ce que** l'agent de collage a été dissous dans un solvant organique, tel que l'acétone.

5. Procédé selon l'une quelconque des revendications 2 à 4, **caractérisé en ce que** la teneur en agent de collage dans la solution ou la dispersion du procédé est de 0,001 à 5 % en poids, de préférence de 0,05 à 0,2 % en poids.

6. Morceau de bois thermiquement modifié pouvant être obtenu par un procédé selon l'une quelconque des revendications précédentes, **caractérisé en ce que** le bois a été imprégné d'un agent de collage hydrophobe, qui est réactif avec la cellulose et au moyen duquel le bois a été rendu hydrofuge, ledit agent de collage étant un dimère d'alkyl cétène (AKD) ayant une chaîne alkyle en C₁₆-C₂₂ et/ou un anhydride d'acide alcényle succinique (ASA) ayant une chaîne alcényle en C₁₆-C₂₂.

7. Morceau de bois thermiquement modifié selon la revendication 6, **caractérisé en ce que** le bois a été imprégné de l'agent de collage afin de répartir uniformément l'agent de collage sur tout le bois.

8. Utilisation d'une colle hydrophobe réactive avec la cellulose dans le traitement d'un morceau de bois thermiquement modifié ayant un nombre de radicaux libres augmenté d'au moins 1,5 fois par la modification par rapport à un bois non traité correspondant, le bois étant imprégné de la colle pour le rendre hydrofuge, ladite colle étant un dimère d'alkyl cétène (AKD) ayant une chaîne alkyle en C₁₆-C₂₂ droite et/ou un anhydride d'acide alcényle succinique (ASA) ayant une chaîne alcényle en C₁₆-C₂₂, et au moins lorsque l'agent de collage est l'ASA, le bois traité est séché et ensuite chauffé à une température de 100 à 140°C pendant 15 à 60 minutes.
